

## UNITED STATES PATENT OFFICE

2,071,306

## BLEACHING

Wilhelm Hirschkind, Berkeley, Calif., assignor to  
Great Western Electro-Chemical Company, a  
corporation of California

No Drawing. Original application May 28, 1935,  
Serial No. 23,850. Divided and this applica-  
tion July 27, 1936, Serial No. 92,848

## 9 Claims.

(Cl. 8-2)

This case is a division of my application Serial No. 23,850 filed May 28, 1935.

This invention relates to the treatment of groundwood or mechanical pulp and more particularly to the manufacture of products from such pulp as newsprint, specialty papers, boards, etc. Groundwood pulp, as is well known in the art, is produced by the mechanical disintegration of wood so that the pulp contains all of the lignins and resins, in fact all of the constituents of the wood. In view of all these compounds being present, the bleaching of groundwood pulp and the production of light paper therefrom presents a difficult problem. In my prior patent Re-  
issue No. 19,470 of February 19, 1935, I have disclosed the use of hydrosulphites as a bleaching agent for this purpose. I have now found that groundwood pulp can be lightened more effectively and permanently by the use of various members of a group of compounds known as sul-  
phoxylates.

The materials disclosed herein are more advantageously employed than those in my application Serial No. 23,850, filed May 28, 1935. In that case I have disclosed the use of addition products of hydrosulfurous acid. These are satisfactory but the materials of this case are less corrosive under the same conditions and give a better brightening or bleach. Representatives of these compounds are given in the following:

Sodium formaldehyde sulphonylate  
Zinc formaldehyde sulphonylate

35 Zinc formaldehyde sulphonylate

$\text{NaHSO}_2\text{CH}_2\text{O}$   
 $\text{ZnSO}_2\text{CH}_2\text{O}$   
 $\text{SOCH}_2\text{OHO}$

$\text{Zn}$   
 $\text{SOCH}_2\text{OHO}$

I do not limit myself to these representatives since, for instance, the formaldehyde in this combination can be substituted by any other aldehydes such as acetaldehyde or any ketone as acetone, or other ketones and the metal, sodium or zinc can be replaced by other metals as for instance potassium, calcium, magnesium or by the ammonium radical. The outstanding characteristics of these compounds are that they are very stable at ordinary temperature and that their bleaching effect is exerted only at high temperatures (above 100° F.) up to the boiling point of water.

In utilizing the process of my invention I either add the compound as a solid, in form of a solution to the material to be bleached or else I form the compound in situ in the material undergoing bleaching. Thus I have bleached groundwood

pulp by adding to the hot pulp at about 180° F. zinc formaldehyde sulphonylate in small amounts. The pulp reduced quickly in color and finished with a considerably lighter and more permanent color than one bleached under similar conditions with hydrosulphite alone or with a hydrosulphite addition compound. I have also successfully bleached groundwood pulp by forming the sulphonylate directly therein by methods well known for manufacture of this material. Zinc formaldehyde sulphonylate can be produced readily from zinc hydrosulphite and formaldehyde by the addition of zinc dust in an acid aqueous medium, or else the addition compound, zinc hydrosulphite formaldehyde, can be treated with zinc dust in an acid aqueous medium. Another method is by treating hydrosulphite with formaldehyde in the presence of an alkali or by treating the addition compound zinc hydrosulphite formaldehyde with an alkali such as caustic soda, caustic potash or ammonia. There are also other combinations possible such as starting out from alkali sulphites or from  $\text{SO}_2$  and treating with zinc dust, thereby forming hydrosulphite as the intermediate product.

In the manufacture of groundwood pulp, good use can be made of the heat generated in the grinding operation by adding the sulphonylate directly to the water which is used in the grinder although the heat source is not limited to this. The temperature in the grinder is usually above 120°, usually 140° F. and may go as high as 200° F. Under these conditions the bleaching process is usually completed in a short time. Depending on the type of pulp and the quality of bleaching agent used it may or may not be advantageous to add a washing step. The treatment to be used may be the same as that disclosed in my pending application, Serial No. 755,929 filed December 4, 1934.

As above indicated high temperature is essential in bleaching with these compounds and by utilizing the heat of the grinding operation this temperature is obtained without any additional cost although the pulp can be heated if desired artificially. The better results obtained with these compounds over inorganic hydrosulphites, especially the greater permanency of the color, easily offset the heating costs so that the bleaching step does not have to be confined to the grinding operation but can be practiced at any point in the flow of the pulp up to the paper machine proper whereat the pulp is hot.

The bleach occurs quickly, usually in less than half an hour. After the bleach, depending on

the material, the pulp may be washed or directly converted into paper. It is to be pointed out that a pulp bleached with a sulphoxylate is many times more stable than one bleached with a hydrosulfite. For example, two batches of the same pulp were bleached at the same time, one with a hydrosulfite and the other with a sulfoxylate. After bleaching they were permitted to remain exposed to the air in their aqueous suspension. The hydrosulfite bleached pulp darkened quickly while the sulfoxylate bleached pulp did not darken until after nearly a week had elapsed.

With some wood pulps it is advantageous to wash after bleaching while with others it is not. The bleach herein disclosed can be substituted for the bleaching operation disclosed in my application Serial No. 755,929 filed December 4, 1934 and the wash can be optional as I have disclosed therein.

In general the bleach of this invention is useful wherever a quick lightening of color is desired at low cost. The materials useful in accordance with this invention are more satisfactory for high temperature bleaching than inorganic hydrosulfites inasmuch as they show a very marked increase in color lightening. This makes them useful in the production of news print from ground wood pulp as well as on press board products of board machines and specialty products. Since the bleach is very quick and yet effective it can be used to advantage on such products particularly as they have to be made at low unit cost because of the competition market existing.

It is an object of the present invention to provide a high temperature bleaching process for ground wood pulp.

Another object of the invention is to provide an improved process for the manufacture of a product of a light color from ground wood pulp.

The invention possesses other objects and features of advantage, some of which, together with the foregoing, will appear hereinafter.

One preferred operation is as follows:

Wood suitable for production of ground wood pulp is passed from storage to a grinder wherein it is mechanically disintegrated. As is usual, the grinder is showered with water and this water stream carries the wood pulp away while cooling the grinder. The pulp stream has a temperature leaving the grinder of between 100° F.-212° F. and usually between 140° F.-180° F. This heat is supplied by the work done in disintegrating the wood, the water shower cooling the grind stone and thus providing the heat for the pulp stream. The temperature of the incoming water stream is usually between 60° F. and 80° F. At these temperatures the sulphoxylate is quite stable and exhibits little activity. It can therefore be manufactured and fed in easily with the water shower. This is particularly so with sulfoxylates for they are not as corrosive as ordinary hydrosulphites or organic addition products of hydrosulphites.

It is generally desirable to perform the bleach operation at a pH on the acid side, usually between 4.5 and 6.5 and preferably between 5 and 6. Suitable inorganic salts can be used to maintain this pH as borax, soda ash, magnesia, and the alkali metal carbonates, bicarbonates, borates, phosphates, sulfites, bisulfites (alkali metal includes sodium, potassium and the am-

monium radical) and calcium sulfite, bisulfite, phosphate or borate.

After the sulphoxylate has been added to the pulp, a short time must be allowed for its action to take place. This is usually only a matter of minutes, the sulphoxylate being added anywhere in the operation. Since the sulphoxylate acts by reduction, the pulp, after its color has been lightened, will darken if the pH is permitted to get much higher than 7.5 on the alkaline side. In connection with pH, the wood pulp is normally acid so that the pulp suspension is usually on the acid side initially. Under these circumstances, acidification need not be resorted to except when only a very alkaline water is available. Precautions against oxidation need not be taken ordinarily since the bleached pulp is quite stable, an unexpected result as well as an advantage over hydrosulphite bleaching which darkens readily on oxidation.

When the bleach has been completed, or while it is going on, the pulp may be subjected to compatible practices as screening, etc. The pulp can be washed after bleaching, if desired; for this a water slightly on the acid side is best used to avoid color reversion due to pH change and to secure the whitest paper. The bleached pulp with its coloring matter reduced can be run directly to the paper machine after its treatment and converted into paper. For this, sizing, coloring matter and diluents, as sulphite pulp, can be added as required.

The sulphoxylate added can be any of the usual sulphoxylates as a formaldehyde sulphoxylate and reaction products of an aldehyde with sulfoxyllic acid or a salt thereof, particularly a metal salt as zinc or an alkali metal, sodium, potassium and ammonia, or one of the alkaline earths, calcium and magnesium. Various aldehydes can be used including acetaldehyde, formaldehyde and any of the other aldehydes or aldehyde compounds. The sulphoxylate can be formed virtually in situ by adding an aldehyde to water carrying a salt of sulfoxyllic acid. Thus, zinc dust and SO<sub>2</sub> can be added to the water. After a short time an aldehyde is added when the mixture is passed to the grinder shower. Instead of an aldehyde a ketone can be used. Both ketones and aldehydes form addition products so that any aldehyde or ketone can be used. The simplest formula for an aldehyde and a ketone is-



where R' is hydrogen for an aldehyde and any organic radical for a ketone wherein a carbon is bonded to the carbon in the formula. Any aldehydic or ketonic compound, aliphatic or cyclic, including carbocyclic as well as heterocyclic, within these formulas can be used as a basis for forming the sulphoxylate.

The invention is applicable to any stock containing an appreciable percentage of ground wood pulp. An example of such a stock is news print stock which is made up of ground wood and sulphite pulps. The problem of lightening color of such a stock is present due to the presence of the ground wood in an appreciable percentage. Such mixed stocks are included and are contemplated in my process and are therefore within the scope of the claims.

I claim:

1. Bleaching ground wood pulp with an organic sulphoxylate at a temperature between 100° and 212° F.

2. Bleaching ground wood pulp with the addition product of a salt of sulfoxylic acid and an aldehyde at a temperature between 100° and 212° F.

3. Bleaching ground wood pulp with the addition product of a salt of sulfoxylic acid and a ketone at a temperature between 100° and 212° F.

4. Bleaching ground wood pulp at a temperature between 100°-212° F. with the addition product of sulfoxylic acid and an organic compound of the formula—



15 where R is any organic radical and R' is hydrogen or any organic radical.

5. Bleaching ground wood pulp at a temperature of about 140° F. with the addition product of sulfoxylic acid and an organic compound of the formula—



where R is any organic radical and R' is hydrogen or any organic radical.

25 6. Bleaching ground wood pulp at a temperature between 100°-212° F. with the addition product of sulfoxylic acid and an organic compound of the formula—



30 where R is any alkyl or aryl group and R' is hydrogen or any alkyl or aryl group.

7. Bleaching ground wood pulp at a temperature of about 140° F. with the addition product

of sulfoxylic acid and an organic compound of the formula—



where R is any alkyl or aryl group and R' is hydrogen or any alkyl or aryl group.

8. Bleaching ground wood pulp at a temperature between 100°-212° F. with the addition product of sulfoxylic acid and an organic compound of the formula—



where R is any organic radical and R' is hydrogen or any organic radical, while maintaining said pulp at a pH substantially between 4.5 and 6.5 by addition of an inorganic alkaline salt effective to maintain said pH substantially between 4.5 and 6.5.

9. Bleaching ground wood pulp at a temperature of about 140° F. with the addition product of sulfoxylic acid and an organic compound of the formula—



where R is any organic radical and R' is hydrogen or any organic radical, while maintaining said pulp at a pH substantially between 4.5 and 6.5 by addition of an inorganic alkaline salt effective to maintain said pH substantially between 4.5 and 6.5.

WILHELM HIRSCHKIND.